

April 3, 1928.

1,665,152

R. M. WITHYCOMBE

PROCESS OF MANUFACTURING BRUSHES

Filed Oct. 2, 1924

FIG. 1



FIG. 2



FIG. 3



Inventor  
Robert Morse Withycombe,

By   
Attorney

## UNITED STATES PATENT OFFICE.

ROBERT MORSE WITHYCOMBE, OF SYDNEY, NEW SOUTH WALES, AUSTRALIA.

## PROCESS OF MANUFACTURING BRUSHES.

Application filed October 2, 1924, Serial No. 741,250, and in Australia May 2, 1924.

This invention relates to a process for making brushes and has for its object a process for manufacturing that type of brush which is composed of a strip of rubber cut into filaments for a portion of its width, the strip being then so aggregated as to bring the filaments closely together into a tuft.

Heretofore it has been found difficult to cut the filaments with any degree of rapidity without distorting them, due to the extreme elasticity, with consequent mobility, of the rubber. A further disadvantage has been that the filaments, when gathered together into a tuft, have sometimes tended to incline outwardly especially when the strip is very thin or the filaments are comparatively long. Further, a brush made according to known processes has not been well adapted that use where it is essential for the brush shall carry a considerable quantity of liquid, because in such brushes the filaments lie closely adjacent to each other and substantially parallel so that there are no decided spaces or interstices between which the liquid may be retained.

I have found, however, that if the filaments are formed with a curved set, the concave side being directed inwardly, the filaments will when the strip is formed into a brush be forced apart in an intermediate portion of the brush forming reservoirs which retain the liquid by surface tension and deliver it to the end of the brush in the usual manner by capillarity.

The process of the present invention concerns itself both with making the cutting of the filaments easy and with imparting to them a curved set which will enable the brush to fulfill the desired function of a reservoir.

## In the drawings:—

Figure 1 represents a brush made according to the process of the present invention, shown in elevation.

Figure 2 is a plan view of a portion of a strip of rubber illustrating the step of cutting the filaments.

Figure 3 is a perspective view of a portion of the rubber strip illustrating the curved set.

According to the invention, I first secure the strip of rubber by means of an adhesive to a temporary base or backing 2 of cardboard or other suitable flexible but comparatively inelastic material. This backing, with the strip of rubber fastened there-

upon is then passed in any suitable manner into operative relation with cutting means by which the slits 3 are formed in the rubber, said slits preferably including parallel portions 4 and inclined portions 5 which intersect the parallel portions thus dividing the strip of rubber into two strips formed with interleaved filaments 6. The cutting of the filaments may be produced in any suitable manner, the slits being formed in a single operation or in successive steps as may be preferred. The whole strip, when so cut, is removed from the backing 2 and pulled apart forming two strips of reduced width, the filaments of each strip being substantially identical in size and shape, said strips forming the stock blank, suitable lengths of which are used for the making of a brush. Each of said strips, when rolled, forms the brush portion which may then be mounted in a suitable handle, or the unslitted part of the strip, when rolled or otherwise aggregated together, may be utilized as the shank or handle. In this part of the process it is to be understood that the adhesion of the strip to the backing prevents the filaments from exercising their property of elasticity while being cut, so that they remain immobile under the cutting means thereby avoiding distortion.

The provision of a curved set in at least the filamentous part of the strip prior to forming it into a brush is one of the steps in the complete process. This may be effected in several ways, one of which is to coat one side of the strip with linseed oil or its equivalent and leave it to dry. The linseed oil in drying shrinks, thus drawing the rubber into a concave form as shown in Figure 3. This effect can also be produced by stretching the rubber upon a saddle-shaped form and coating it with any suitable composition by means of which a differential tension is produced on opposite sides of the strip. The curved set may also be imparted to the strip by vulcanizing the rubber, prior to cutting the same, upon a suitable form in the manner in which the inner tubes of automobile tires are produced. When the strip having the curved set is rolled with the concave sides of the filaments directed inwardly the brush assumes the form shown in Figure 1 in which the ends of the filaments oppose each other, causing the intermediate portion of the brush to bulge as shown at 7 in Figure 1, thereby forming inter-filamentous spaces of substan-

tial capacity constituting reservoirs in which the liquid is retained by surface tension. These reservoirs have the form of widened interstices converging toward the lower end 5 of the brush. This permits liquid from the intermediate portion of the brush to be drawn to the end of the brush by capillarity.

Although I have here outlined what I believe to be a practical and efficient process 10 for accomplishing the desired results it is to be understood that such changes can be made in the process or in the sequence of the steps thereof as to not depart from the invention as claimed.

15 Having described my invention what I claim as new and desire to secure by Letters Patent, is:—

1. The process of making a filamentous rubber blank which consists in uniting one 20 entire face of a strip of flexible elastic rubber to a relatively non-elastic backing, cut-

ting said strip with slits while it is united to said backing, forming filaments, and removing said backing.

2. The process of making a rubber brush 25 which consists in causing a strip of flexible elastic rubber to adhere to a transversely curved relatively non-elastic backing, treating said strip while in adherence with said backing, to give it a curved set determined 30 by the curvature of said backing, bringing said backing with the adhered rubber, into operative relation with suitable cutting means to slit the rubber without distortion, forming filaments, removing said backing 35 and rolling the strip with the concaved side directed inwardly to bring the elements together into a tuft having the points thereof directed toward the axis of said tuft.

In testimony whereof I have hereunto set 40 my hand.

ROBERT MORSE WITHYCOMBE.